

F. H. F. HAMPTON.  
SMELTING PROCESS AND APPARATUS.  
APPLICATION FILED MAR. 30, 1916.

1,315,551.

Patented Sept. 9, 1919.



F. H. Franklin Hampton

By Albert F. Nathan, Attn.

# UNITED STATES PATENT OFFICE.

FRANK H. FRANKLIN HAMPTON, OF SEWELL, CHILE, ASSIGNOR OF ONE-HALF TO W. W. STENNING, OF LONDON, ENGLAND.

## SMELTING PROCESS AND APPARATUS.

1,315,551.

Specification of Letters Patent.

Patented Sept. 9, 1919.

Application filed March 30, 1916. Serial No. 87,736.

*To all whom it may concern:*

Be it known that I, FRANK HOWARD FRANKLIN HAMPTON, a subject of Great Britain, and residing at Sewell, Rancagua, Chile, have invented a new and Improved Smelting Process and Apparatus, of which the following specification is a full disclosure.

This invention deals with an improved system for effecting metallurgical operations and, in this preferred more concrete aspect, it proposes a process especially adapted for smelting a finely divided product, as well as an apparatus instrumental in carrying out said process.

One object within the contemplation of this invention is to render available a system comprehending a novel process and apparatus whereby any finely divided concentrate or ore such as that recovered by the flotation process, may be automatically and continuously smelted to matte and slag by means of heat derived from the combustion of any fuel capable of atomization.

Another object is to organize a process such that a finely divided ore may, without being briqueted, be efficiently smelted by means of pulverized coal which is unsuitable for ordinary conditions of combustion.

Another object is to create a smelting structure of a simple and comparatively inexpensive design whereby a finely divided product may be continuously and efficiently smelted and whereby the herein disclosed process may be effectively carried out.

Various other objects and advantages will be in part obvious from the annexed drawings and in part indicated in connection therewith by the following analysis of this invention.

This invention accordingly consists in the features of construction, combinations of parts and in the relative proportioning and disposition thereof and in the unique relations of the various steps and operations, all as more completely outlined herein.

To enable others skilled in the art so fully to comprehend the underlying features thereof that they may embody the same by the numerous modifications in structure and relation contemplated by this invention, drawings depicting a preferred form of my proposed apparatus have been annexed as a part of this disclosure, and in such drawings, like characters of reference denote corre-

sponding parts throughout all the views of which:

Figure 1 represents in vertical median section a furnace embodying this invention. Fig. 2 is a horizontal section of said furnace taken along line B—B of Fig. 1, and Fig. 3 is a fragmentary vertical radial section taken along line C—C of Fig. 2.

Continuing now by way of a more detailed description of the shown exemplification of this invention it may be primarily noted that one of the prominent characteristics of this process resides in performing the smelting reactions while the material is in a dispersed state of suspension in a gaseous blast. The particles are individually smelted in a comparatively isolated condition and subsequently agglomerate to form a bath of slag and matte.

Metallurgists have heretofore carried out their smelting operations *en masse*, and all conditions have accordingly been so adjusted that the presence or formation of finely divided material has constituted a serious disrupting factor. In dealing with a product of a pulverulent nature *ab initio*, considerable preparatory expense was incurred by attempts to briquet or otherwise bring the product into a bulky condition.

My invention, however, proposes to proceed directly with the smelting of the product while it is in its pulverulent condition and to employ cheap pulverulent fuel in doing so. To that end it establishes zones of temperatures progressively varying in accordance with the progress of the metallurgical reactions and to cause the particles to project or gravitate through said temperature zones while simultaneously subjected to smelting conditions so that said particles may ultimately gravitate or rain down in the form of slag and matte to coalesce with a bath formed thereby.

Preferably, the temperatures and smelting conditions are established by correctly proportioning air and atomized fuel in relation to the composition of the charge so that complete combustion of the fuel will be had as a result of the combined oxidizing effects of the air and of the charge. These materials are projected into a smelting chamber in the form of a blast carrying the particles in a state of suspension and permitting them in the chamber to gravitate through the

60

65

70

75

80

85

90

95

100

110

flame in more highly heated portions of the gases which are deflected by the walls of the chamber so as to control this action.

This may best be understood by referring 5 to the drawings showing an upstanding cylindrical smelting chamber *a* formed of magnesite brick or other available heat resisting material and preferably having a removable dome shaped top and providing 10 parts for the entry of the combustion and smelting ingredients and for the withdrawal of the products of combustion and smelting. Thus, the lower portion of the smelting chamber *a* is provided in its center with an 15 upstanding charging twyer *c* which is directed upwardly coaxially with the chamber and which upstands sufficiently in the nature of a nozzle to provide for a collection receptacle *b* forming a hearth for containing the 20 bath of matte and slag and permitting the same to be tapped off at any convenient point by means of the furnace spout *q* shown in Fig. 3 and thence to the settler in the pit *r*.

25 This charging twyer *c* may be utilized for supplying the chamber not only with air and the pulverulent charging material, but also with sufficient carbon in the nature of pulverulent fuel to form the requisite heat 30 by burning with the air and under the influence of this heat to also combine with the oxidizable ingredients in the charge to smelt the same. Either solid, liquid or gas fuel may be used, or any mixture of 35 any two; and a change from one to either may be effected without disturbing the continuity of the furnace operation, or without changing the conditions of the smelting chamber. Should solid fuel be used, it may be initially or further pulverized and automatically and continuously fed into the blast and fuel main *m*, or through the feed opening *n* by means of an adjustable feeder; and if oil or gas fuel be used it may be 45 delivered to a suitable burner *o* by means of a pipe *p*.

Only the exact amount of air required for the complete combustion of the fuel elements is used for the blast. This blast air is 50 drawn through the blast air heating jacket "h" by a conventional blower and is delivered through the blast and fuel main "m" at a temperature sufficient to deliver the charge to the smelting chamber at a temperature of about 500 deg. C.

The material to be smelted, such as concentrate from the flotation process of recovery or any other finely divided concentrate or ore, is automatically and continuously fed through the feed opening "n" by any conventional means. The charge together with its correct proportion of air and fuel, becoming perfectly mixed, is projected into the smelting chamber through the charge and blast twyer "C" in the form of a dust

cloud, at a temperature of about 500 deg. C. and is ignited by the heat thrown off from the brickwork surrounding the twyer. This dust cloud enters the smelting chamber, at a relatively high velocity. Owing to expansion the air very soon loses part of its initial velocity, but the larger particles of solids, by virtue of their momentum rise upward in the central current of flame until overcome by gravity their direction changes 70 and they follow the descending current of gases, being on their downward journey subjected to the heat radiated from the central column of flame and heat reverberated from the encircling brick walls. The formation 75 of any considerable amount of flue dust is prevented by the particles of solids, together with any ash from the fuel being forced through the zone of highest 80 temperature where they will fuse and fall 85 to the hearth and assume their respective places in the matte and slag.

The temperature of the charge being about 500 deg. C. all moisture present will be instantly changed to water vapor and directly after any combined water will be 90 evaporated. When the temperature of 700 deg. C. is reached,  $FeS_2$  will change to  $FeS$  and  $S$ , the latter being oxidized instantly to  $SO_2$ , and if solid fuel be present, some  $SO_2$  95 may react as follows:— $SO_2$  plus  $C=S$  plus  $CO_2$  plus 27,940 cals. As the charge finely divided and carried upward by the current of air reaches a higher temperature of 900 deg. to 1000 deg. C. the  $FeS$  will be oxidized 100 to  $FeO$  plus  $SO_2$ , and simultaneously the former will unite exothermically with the  $SiO_2$  of the charge thus forming the slag. The minute spray of matte and slag thus 105 formed will fall slowly to the bottom of the smelting chamber, with the descending gases at the side, or will collect on the sides of the smelting chamber and trickle slowly to the bottom. Any  $CaO$  present will be 110 melted and then absorbed by the  $FeO$ ,  $SiO_2$ , mixture forming a ferro-calcic silicate slag. The mixture of slag and matte at the bottom 115 will separate slowly as in the fore-hearth, but if tapped constantly a fore-hearth must be used.

As the pulverized charge enters the blast which has been previously heated to a temperature sufficiently high to raise the temperature of the total charge to 500 deg. C. before it reaches the furnace proper, the 120 first event to take place is the evaporation of all moisture present to water vapor. Any combined water present will be evaporated next.

The CO formed by the fuel on first entering the smelting chamber will reduce  $CuO$  to  $Cu$ , according to the equation  $CuO$  plus  $CO= Cu$  plus  $CO_2$ , and the blast will be regulated to oxidize only the C and no S, and as the charge ascends in the smelting 125 130

- chamber to a point where a temperature of about 900 deg. C. is reached, the formation of the slag in the form of a spray commences; the constituents of the slag being 5 essentially the FeO and SiO<sub>2</sub> in the charge, together with any CaO and Al<sub>2</sub>O<sub>3</sub> which may be present. Any CuS entering the furnace will first be more or less oxidized to CuO. Scorification of the metallic copper 10 is prevented by sulfurizing the Cu to Cu<sub>2</sub>S by means of the FeS present according to the equation 2Cu plus FeS=Cu<sub>2</sub>S plus Fe. The Fe thus formed being slagged simultaneously by the SiO<sub>2</sub>. The slag and matte 15 collect in the bottom of the smelting chamber as in the case of partial pyritic smelting previously quoted.
- Without further analysis, the foregoing will so fully reveal the gist of this invention 20 that others can by applying current knowledge readily adapt it for various applications without omitting certain features that, from the standpoint of the prior art, fairly constitute essential characteristics of the 25 generic or specific aspects of this invention, and therefore such adaptations should and are intended to be comprehended within the meaning and range of equivalency of the following claims.
- 30 Having thus revealed this invention, I claim as new and desire to secure the following combinations of steps and elements, or equivalents thereof, by Letters Patent of the United States:—
- 35 1. A smelting process which comprehends projecting a finely-divided self-fluxing material upwardly into a zone sufficiently heated to cause the formation of melted slag; permitting the melted globules to coalesce to form a bath of slag and valuable 40 products, and causing all the gases to escape at the base only of said zone.
2. A smelting apparatus combining a smelting chamber having a closed top; means for maintaining the same at a smelting temperature; means for projecting self-fluxing material into said chamber in dispersed form, whereby the same may be smelted; 45 outlets for the gas located at the base of said chamber and means for collecting the molten 50 products.
3. A smelting process which comprehends causing a finely-divided self-fluxing material together with gas to uprise and descend together with the gas through a high temperature zone to be smelted therein in a state of sub-division; and then permitting the particles to coalesce to form a bath of slag and matte. 55
4. A smelting apparatus combining an upright smelting chamber having gas outlets only adjacent its lower end and also providing for the drainage of molten products; and means for projecting upwardly into said chamber a flame suspending particles of a 60 self-fluxing mixture. 65
- In witness whereof, I hereunto subscribe my name, as attested by the two subscribing witnesses.
- F. H. FRANKLIN HAMPTON.
- Witnesses:
- J. F. McGUIRK,  
JOHN GARVIN.